

Jan. 8, 1935.

C. F. LAUENSTEIN

1,987,481

PROCESS OF METAL TREATMENT

Filed Feb. 17, 1930

3 Sheets-Sheet 1

Fig. 1.



Fig. 2.



Inventor  
Carl F. Lauenstein  
by Parker + Carter  
Attorneys.

Jan. 8, 1935.

C. F. LAUENSTEIN

1,987,481

PROCESS OF METAL TREATMENT

Filed Feb. 17, 1930

3 Sheets-Sheet 2

*Fig. 3.*



*Fig. 4.*



Inventor  
Carl F. Lauenstein  
by Parker + Carter  
Attorneys.

Jan. 8, 1935.

C. F. LAUENSTEIN

1,987,481

PROCESS OF METAL TREATMENT

Filed Feb. 17, 1930

3 Sheets-Sheet 3

Fig. 5.



Inventor  
Carl F. Lauenstein  
by Parker & Carter  
Attorneys.

## UNITED STATES PATENT OFFICE

1,987,481

## PROCESS OF METAL TREATMENT

Carl F. Lauenstein, Indianapolis, Ind., assignor  
to Link-Belt Company, Chicago, Ill., a corpora-  
tion of Illinois

Application February 17, 1930, Serial No. 428,952

12 Claims. (Cl. 148—21.8)

This invention relates to the problem of annealing a ferrous alloy and has for one object to provide a means for accomplishing the complete cycle of annealing rapidly. Other objects will appear from the time to time in the specification and claims.

The invention may be applied to the manufacture of malleable castings and it will be described herewith as so applied. The iron alloy most generally used for castings which are to be malleabilized is known usually as white iron and it consists mainly of iron and carbon. It may also contain, among other things, silicon, manganese, sulphur, phosphorus and relatively small amounts of impurities. After the casting operation is completed all, or practically all, of the carbon is in combination with the iron in the form of iron carbides. The general object of the annealing operation is to throw the carbon out of combination with the iron so that after the annealing the carbon is in the form of globules or crystals, separate from and interspersed between the crystals of the ferrite.

The following drawings illustrate various stages in the manufacture of the metal which forms the subject of the present invention. They are drawings made in reproduction of microphotographs.

Fig. 1 illustrates white cast iron;

Fig. 2 is a similar view showing the iron after it has been heated for four hours at 1650° F.;

Fig. 3 is the iron after it has been heated for four hours at 1650° F. and four hours at 1850° F.;

Fig. 4 is iron after it has been heated four hours at 1650° F. and 4 hours at 1850° F., and cooled to a point below the critical temperature, approximately 1375° F.;

Fig. 5 is the finished product after it has received the two heatings above mentioned and after it has been cooled first to approximately 1400° F., then at a controlled rate of speed to 1200° F. and subsequently cooled to room temperature.

In Fig. 1 the relatively white areas A are cementite and the gray or relatively dark areas B are an iron carbide in the form of pearlite, sorbite or troostite, depending on the rate at which the casting was cooled.

In Fig. 2 the white areas A have decreased. They still represent cementite. The gray areas still indicate iron carbide and certain darker areas C have appeared. These are graphitic carbon.

In Fig. 3 the black areas C have increased in size and the white has disappeared. The black

areas represent, as before, carbon; the gray areas B represent iron carbide.

In Fig. 4 the black areas C of carbon have increased somewhat, the gray area represents iron carbides and the white area D represents ferrite from which all of the carbon has been removed. 5

Fig. 5, representing as it does the finished product, shows widely diversified and relatively small black areas C of carbon and the remainder of the body of the metal is made up essentially 10 of white areas D which are ferrite grains.

In the past the malleabilizing process has been slow. The iron has been normally heated to approximately 1650° F. This does not throw all of the carbon out of combination with the 15 ferrite. It thus does not remove all of the iron carbide. The iron is raised to the heat mentioned and held there sufficiently long to permit whatever chemical change which can take place to take place. The casting is then cooled to 20 about the critical temperature, somewhere between 1350° F. and 1375° F. As a result of this cooling a further quantity of the carbon is thrown out of combination. However, an appreciable residue of carbon still remains in combination. 25 The usual method of getting this final residue out of combination is to cool extremely slowly through the critical range, the rate of cooling being about 5° F. per hour and this final stage frequently requires as much as 48 hours. 30

Experiments have shown that by increasing the temperature of the initial heating above 1650° F. the carbon can be thrown out very much more rapidly and the process greatly shortened and, within certain limits, the higher the 35 heat the greater the rapidity with which the initial or partial breaking down of the iron carbide may be accomplished, for example, the time required when the metal is heated to approximately 1850° F. is something less than one-third 40 that required when it is heated to only 1750° F.

It was found, however, that the carbon, when thrown off as the result of this high heat, when heated to this temperature rapidly, takes on a peculiar form. Instead of being in the form of 45 a relatively large number of relatively small globules or balls, carbon is found in a relatively small number of relatively large irregularly shaped, angularly formed bodies with points running out from the main body and penetrating between the ferrite grains. Such a carbon formation reduces the strength and ductility of the finished product. Probably this is caused by the fact that when the carbon is precipitated at such a high rate of speed, it cannot form small areas 50 55

but forms rather into a relatively few large, irregularly shaped areas or bodies. It is one of the objects of this invention to avoid the defect just mentioned and to secure the benefit of the rapid speed by the use of the high temperatures while causing the carbon, when precipitated out, to take the better form of a relatively larger number of rounder or more nearly ball shaped areas or bodies.

10 The solution of the difficulty above indicated was found by heating the metal preferably at a rapid rate, first to approximately 1650° F. and holding it at that temperature for a relatively short period, in one example, for four hours; subsequently the metal was heated to 1850° F. approximately, and was held at that temperature for a short period, for example, about four hours; it was then cooled to about 1400° F. and held at that temperature for the time necessary to allow the temperature to equalize itself throughout all the material being treated, in one example this was approximately one hour; after that it was cooled to approximately 1200° F. at a controlled rate which may be about 8° F. per hour. It was found that by this heat treatment a satisfactory malleable iron was formed and that the carbon appeared in a large number of bodies and that these were of a satisfactory form and shape. The time required under this method for the complete cycle of annealing, is in the neighborhood of 37 hours as compared to the usual seven or eight days for a complete annealing cycle by the method now generally practiced in the art.

It is believed that this method, which has proved in practice to be successful and, as indicated, greatly reduces the time required for the complete annealing cycle, operates in the following steps: The metal is first heated to approximately 1650° F. and held at that temperature about four hours. This heating, while not sufficient to throw out of combination all of the carbon, which can be thrown out at that temperature, is sufficient to throw out some of it and there is thus formed a large number of relatively small carbon nuclei. The metal is then heated to a higher temperature, approximately 1850° F. The remaining carbon is rapidly thrown out of combination and, due to the fact that a large number of carbon nuclei has already been formed at the lower temperature, this additional carbon now thrown out at the higher temperature goes into the nuclei already formed and the final result is that the metal embodies a large number of small carbon bodies of satisfactory form and shape, rather than the very few large bodies formed where the first heating is carried out at the extremely high heat.

I claim:

1. The process of heat treating white cast iron to precipitate the carbon which includes heating to approximately 1650° F., holding at that temperature for a time sufficient partially to precipitate the carbon and to cause it to form into a relatively large number of relatively small, widely dispersed carbon nuclei, heating to approximately 1850° F., holding at that temperature for a time sufficient to complete the precipitation of the remaining carbon into the nuclei so formed, cooling to approximately 1400° F. and holding at that temperature for a time.

2. The process of heat treating white cast iron to precipitate the carbon which includes heating to approximately 1650° F., holding at that temperature for a time sufficient partially to precipitate the carbon and to cause it to form into

a relatively large number of relatively small, widely dispersed carbon nuclei, heating to approximately 1850° F., holding at that temperature for a time sufficient to complete the precipitation of the remaining carbon into the nuclei so formed, cooling to approximately 1400° F., holding at that temperature for a time, and subsequently cooling to approximately 1200° F. at a controlled rate of cooling.

3. The process of heat treating white cast iron to precipitate the carbon which includes heating to approximately 1650° F., holding at that temperature for a time sufficient partially to precipitate the carbon and to cause it to form into a relatively large number of relatively small, widely dispersed carbon nuclei, heating to approximately 1850° F., holding at that temperature for a time sufficient to complete the precipitation of the remaining carbon into the nuclei so formed, cooling to approximately 1400° F., holding at that temperature for a time, and subsequently cooling to approximately 1200° F., at a rate of approximately 8° F. per hour.

4. The process of heat treating white cast iron to precipitate the carbon which includes heating to approximately 1650° F., holding at that temperature approximately four hours, heating it to approximately 1850° F., holding at that temperature for a substantially equal period, cooling to approximately 1400° F., and holding at that temperature for a less period.

5. The process of heat treating white cast iron to precipitate the carbon which includes heating to approximately 1650° F., holding at that temperature approximately four hours, heating to approximately 1850° F., holding at that temperature for a substantially equal period, cooling to approximately 1400° F. and holding at the temperature of 1400° F. for approximately one hour.

6. The process of heat treating white cast iron to precipitate the carbon which includes heating to approximately 1650° F., holding at that temperature approximately four hours, heating it to approximately 1850° F., holding at that temperature for a substantially equal period, cooling to approximately 1400° F., holding at that temperature for a less period, and cooling from said last mentioned temperature at a controlled rate of cooling.

7. The process of heat treating white cast iron to precipitate the carbon which includes heating to approximately 1650° F., holding at that temperature approximately four hours, heating it to approximately 1850° F., holding at that temperature for a substantially equal period, cooling to approximately 1400° F. and holding at the temperature of 1400° F. for approximately one hour, and cooling from said last mentioned temperature at a controlled rate of cooling.

8. The process of heat treating white cast iron to precipitate the carbon which includes heating to approximately 1650° F., holding at that temperature approximately four hours, heating it to approximately 1850° F., holding at that temperature for a substantially equal period, cooling to approximately 1400° F. and holding at that temperature for a less period, and cooling from said last mentioned temperature at approximately 8° F. per hour until a temperature of approximately 1200° F. is reached.

9. The process of heat treating white cast iron to precipitate the carbon which includes heating to approximately 1650° F., holding at that temperature approximately four hours, heating it to approximately 1850° F., holding at that tempera-

ture for a substantially equal period, cooling to approximately 1400° F. and holding at the temperature of 1400° F. for approximately one hour, and cooling from said last mentioned temperature at approximately 8° F. per hour until a temperature of approximately 1200° F. is reached.

10. The process of heat treating white cast iron to precipitate the carbon which includes heating to approximately 1650° F., holding at that temperature approximately four hours, heating to approximately 1850° F., holding at that temperature for a substantially equal period, cooling rapidly to approximately 1400° F., and holding at that temperature for a less period, cooling from 15 said last mentioned temperature at approximately 8° F. per hour until a temperature of approximately 1200° F. is reached and subsequently cooling to room temperature at an uncontrolled rate of speed.

20 11. The method of heat treating white cast iron

to precipitate the carbon, which includes heating the metal to and holding it at a temperature sufficient to precipitate some of the carbon relatively slowly to form a relatively large number of relatively small carbon nuclei and subsequently heating the metal to and holding it at a higher temperature to precipitate substantially all of the remaining available carbon.

12. The method of producing malleable cast iron which comprises the steps of heating white cast iron to a temperature of approximately 1650° F., holding the casting at that temperature for a few hours, heating the casting to a temperature of approximately 1850° F., holding it at that temperature for a few hours, cooling the casting to a temperature of approximately 1400° F., holding it at that temperature for a few hours, and then further cooling the casting.

CARL F. LAUENSTEIN. 20